

# UNITED STATES PATENT OFFICE.

EDOUARD PAUL LOUIS SISLEY, OF LYON, FRANCE, ASSIGNOR TO SOCIETA ANONIMA COOPERATIVA PER LA STAGIONATURA E L'ASSAGGIODELLE SETE ED AFFINI, OF MILAN, ITALY, A CORPORATION OF ITALY.

## PROCESS OF TREATING SILK.

No. 878,902.

Specification of Letters Patent.

Patented Feb. 11, 1908.

Application filed January 16, 1906. Serial No. 296,426.

*To all whom it may concern:*

Be it known that I, EDOUARD PAUL LOUIS SISLEY, chemist, a citizen of the Republic of France, and a resident of 58 Cours Morand, 5 Lyon, France, have invented certain new and useful Improvements in Processes of Treating Silk, of which the following is a specification.

This invention has reference to a novel 10 process of treating silks and pertains particularly to a process of treating silks which have been impregnated, for instance, with salts of tin, for the purpose of preventing spontaneous changes to which such silk 15 yarns, woven fabrics, or goods are subject when exposed to light, heat, and atmospheric influences. Accordingly, this process is applied after the silks have been impregnated with the salts. Heretofore silk has been 20 treated for this purpose with a dilute solution of sulfocyanic acid or its salts.

It is the special object of this invention to provide a process for obtaining a higher degree of tensile strength and elasticity of the 25 silks quicker and in a more satisfactory manner than with the above mentioned substances. I have discovered that thio-urea, its salts, and derivatives are compounds by the use of which this desirable result is obtained.

In carrying out my novel process I substantially proceed as follows. The dyed skeins or hanks of silk are immersed in a dilute solution of thio-urea, its salts, or derivatives to which solution may be added a 35 small quantity of an acid, for instance 2 grams of citric acid per liter of the solution, in order to maintain the scroop or crisp sound while the skeins or hanks so treated 40 are exposed to the air and dried. The quantity of thio-urea, its salts, or derivatives employed in such a bath may vary 10 grams of thio-urea per liter may be used. Woven fabrics likewise may be treated by immersing 45 them in a bath of the above named substances or the solution may be sprayed thereon or any other suitable method may be employed to impregnate the woven fabrics with a solution of the above described chemical agents. The solution of thio-urea may also be mixed with various sizes and the treatment of the goods with thio-urea in combination with the known methods of sizing whereby the goods are at 55 once finished likewise is a feature of this

invention and comes within the scope of same.

The novel process of treating silks with thio-urea imparts to the impregnated yarns of fabrics a high degree of resistance to the 60 action of atmospheric influences but without presenting the deficiency of fabrics which are affected by rust marks. The novel process further imparts to the goods the property of resisting perspiration whereby the formation 65 of stains is prevented in the single threads or fabrics while under the influence of perspiration or of substances containing chlorids. The protecting effect of this treatment is explained by the fact that thio-urea, its salts, 70 and derivatives are more easily oxidized than the silk fiber in the presence of metallic salts such as tin salts leaving then the fiber in a condition of unimpaired strength and increasing its elasticity. The color of the 75 silk fibers thus treated is not affected and remains constant. Tests made with the serimeter verified this statement.

Having thus described my invention I claim as new and desire to secure by Letters 80 Patent:

1. Process of increasing the tensile strength and elasticity of silks weighted with metallic salts consisting in immersing the silks in a slightly acidulated bath of thio-urea compounds, and drying same on the fiber.

2. Process of increasing the tensile strength and elasticity of silks weighted with tin salts consisting in immersing the 90 silks in a slightly acidulated bath of thio-urea and drying same on the fiber.

3. Process of increasing the tensile strength and elasticity of silks weighted with tin salts consisting in immersing the 95 silks in a dilute solution of thio-urea slightly acidulated with citric acid, and drying same on the fiber.

4. Process of increasing the tensile strength and elasticity of silks weighted 100 with tin salts consisting in immersing the silks in a dilute bath of thio-urea slightly acidulated with citric acid and containing sizes, and drying same on the fiber.

Signed at Lyons this 18th day of December, 1905.

EDOUARD PAUL LOUIS SISLEY.

Witnesses:

MERIN VACHON,  
SAUL VEYRE.